

## UNITED STATES PATENT OFFICE.

GEORGE CROMPTON, JR., OF WORCESTER, MASSACHUSETTS.

## COATING TEXTILES WITH METAL.

No Drawing.

Application filed August 26, 1925. Serial No. 52,684.

*To all whom it may concern:*

Be it known that I, GEORGE CROMPTON, Jr., a citizen of the United States, residing at Worcester, in the county of Worcester and Commonwealth of Massachusetts, have invented a new and useful Improvement in Coating Textiles with Metal, of which the following is a specification.

My invention relates to the metal coating of cloth and other textiles. It is possible, as is well known, to print any desired design in an almost unlimited range of colors on cloth. It is also possible to weave many and various designs in different colors by using a multiple shuttle box loom to throw different colored filling and a jacquard machine. The results in the two cases are, however, substantially different; in the latter case the design inheres in the weave itself, while in the former, the lines of division are sharper, as the lines of division have nothing to do with the weave.

Both methods have their peculiar advantages and artistic qualities and will, undoubtedly, always coexist. When manufacturers desired to produce a design in metal on cloth simulating silver or gold, the multiple box loom and the jacquard were resorted to, one class of filling or warp threads, and sometimes both, being twisted with a flat metal wire. Also, paralleling the printing of cloth, bronze and silver powders have been made to adhere to cloth by an adhesive. The trouble with this last process is that the "printing" rolls quickly become clogged with the adhesive substance, and then the resulting design becomes imperfect.

Recently it has been found that a cloth woven without any design and presenting an unbroken face of imitation gold or silver, can be given a design by a deforming process, as the metal will take a certain set.

From all the above my invention clearly distinguishes itself. My invention contemplates the coating of cloth, or other textile, with metal that firmly adheres, yet no adhesive substance is used. Subsequently, I cause this metal coating to lose its rigidity and become pliable.

Referring now particularly to the specific embodiment of the invention in the best form known to me, the first step consists in providing a suitable stencil device having any desired design. A suitable back plate or table is then provided and the cloth is clamped between the two. The result is that the cloth

is completely covered except for those portions on which the coating is to be applied. The back plate and the stencil plate should be firmly fastened together as by the ordinary wood clamps, so that all portions of the cloth adjacent the gap where the metal is to be deposited will be firmly held.

The next step in my process consists in applying the metal in the form of a molten spray. For this purpose, a machine of the general class shown by United States Letters Patent No. 1,100,602, to E. Morf of Zurich, Switzerland, is desirably used. Such a machine fuses metal and then atomizes it, and projects the atomized metal in the form of a spray. The particular machine mentioned will be found fully described in said Letters Patent, but briefly it comprises a small machine adapted to be held in the hand, having a compressed air driven turbine which, through reduction gearing, feeds wire to a fusing nozzle. At the nozzle a hot flame is maintained, the flame being produced by a mixture of combustible gas and compressed air. The exhaust from the air turbine also leads to the nozzle and produces the atomizing and spraying referred to.

I do not claim to be the first to discover the general fact that cloth can be thus sprayed with a molten spray without burning the cloth. Such a conclusion is suggested by United States Letters Patent No. 1,128,058, to M. U. Schoop of Hongg, Switzerland. I have found that by using that above described machine shown in the United States Patent No. 1,100,602, and by using a wire composed of a metal of low fusing point (e. g., tin) that the finest silks and satins can be successfully coated, and that moreover the coating will not peel off.

At this stage in the process, after spraying through all the stencils so that the cloth is completely covered, and desirably stopping before too thick a coating is deposited in any one place, the cloth should be removed and, if desired, a new section treated in the same manner.

At the completion of the coating operation, the cloth has one or a plurality of metal coated portions, arranged in whatever design was desired. The lines of demarcation between the treated and the untreated cloth are sharp. There is, however, an undesirable stiffness to these plated portions and they lack lustre, and it is with the removal of these defects that my invention

is chiefly concerned. To this end the metal that is sprayed onto the cloth must be one that will amalgamate with mercury or with a substance having like properties. Tin, 5 already mentioned, is such a metal.

The cloth, or other textile, having been coated in whole or in part with the non-mercuric metal, is then placed in a bath of mercury, or mercury is allowed to flow over 10 it. The mercury amalgamates with the metal coating, thus forming an amalgam. This step in my process may be hurried by 15 a slight rubbing, but the rubbing is not indispensable, and merely serves to accelerate the action.

The cloth, or textile, should then be brushed to remove small globules of mercury and the article is then complete.

I have found, as aforesaid, that the finest 20 of silks can be thus coated with amalgam in any desired design. The amalgam coating is extremely pliable and the design is sharply defined. It can indeed be removed 25 in part by scraping, but a residuum will always be left that tenaciously adheres to the cloth. Moreover this feature enhances the artistic quality of the resulting product, for 30 the amalgam coating presents different degrees of lustre in different places somewhat in the nature of water marks on paper. The design has a distinctly hand wrought effect, for although several reproductions from a given stencil will have identical configurations, they will lack the monotony of exact 35 sameness.

I have found that the amalgam retains 40 its adherence to the cloth apparently indefinitely. Whereas, if allowed to remain untouched for considerable time it will somewhat lose its lustre, upon being touched or moved about, it regains it.

Cloth thus coated with metal has, as 45 aforesaid, an appearance different from anything heretofore produced. It may be used to advantage, for dress goods, hats, or wall hangings. Other uses will suggest

themselves almost without end to persons interested in such matters.

Such textiles as braids and tassels may be 50 completely coated with amalgam, there being no need to use a stencil in such cases.

Having thus described my process and my product or article of manufacture and given illustrative embodiments of each, I 55 wish it understood that such description is not to be taken in a limiting sense, the scope of my invention being set forth in the following claims, in which the words mercury, amalgam, etc., are to be understood to denote any substance having the same affinitive property as mercury and any alloy having the properties of an amalgam.

I claim:

1. The process of coating a textile with an 65 adhering amalgam, which consists in causing a coating of non-mercuric metal to be deposited on said textile, and then bringing the coating in contact with mercury.

2. The process of coating a textile with 70 an adhering amalgam, which consists in spraying the textile with a non-mercuric metal, and bringing the thus formed metal coating in contact with mercury.

3. The process of coating a textile with 75 an adhering amalgam, which consists in causing a coating of non-mercuric metal to be deposited on said textile in the form of a design, and then bringing the coating in contact with mercury.

4. The process of coating a textile with 80 an adhering amalgam in the form of a design, which consists in spraying the textile with a non-mercuric metal through a stencil, and then bringing the thus formed metal coating in contact with mercury. 85

5. As a new article of manufacture, a textile product having an adhering coating of amalgam.

6. As a new article of manufacture, cloth 90 having a design thereon comprising a broken coating of adhering amalgam.

GEORGE CROMPTON, JR.